

Aug. 28, 1934.

P. P. ALEXANDER

1,971,804

METHOD AND APPARATUS FOR SPRAYING POWDERED MATERIAL

Filed Dec. 4, 1929

Fig. 1.



Fig. 2.



Inventor:  
Peter P. Alexander,  
by *Charles E. Tullar*  
His Attorney.

## UNITED STATES PATENT OFFICE

1,971,804

METHOD AND APPARATUS FOR SPRAYING  
POWDERED MATERIALPeter P. Alexander, Marblehead, Mass., assignor  
to General Electric Company, a corporation of  
New York

Application December 4, 1929, Serial No. 411,634

7 Claims. (Cl. 91—70.1)

The present invention relates to an apparatus and method for spraying powdered material and more particularly hard metal compositions of the character described in Schröter Patents Nos. 1,549,615 and 1,721,416 onto a supporting or foundation metal body. The product disclosed in these patents consists generally of a carbide of an element of the 6th group of Mendelejeff's periodic table, such as tungsten carbide, and an auxiliary 5 binder or cementing metal of the iron group, such as cobalt. These materials are usually mixed together in powdered form, pressed into a desired shape under high pressure and then heated to the sintering temperature of the mixture which may be in the neighborhood of 1380° C. but will vary according to the composition employed. The finished product is usually brazed or welded to a supporting member and thereafter commonly employed as a metal cutting tool or die.

According to the present invention, powdered hard metal compositions of the character disclosed in the above Schröter patents are superheated and sprayed directly onto a supporting metal member thereby providing a uniform layer 10 of hard metal which is suitable for use either as a wear resisting surface or as a metal cutting tool.

In spraying materials of this character, it is desirable to prevent oxidation of the sprayed material as otherwise its physical properties are adversely affected. It is also necessary to control carefully the temperature to which the powdered materials are heated. I have found that the temperature employed should be high enough to cause melting of the binder element, i. e. cobalt. It should not however be high enough to melt the tungsten carbide since melting will alter considerably its physical properties.

The novel features which are characteristic of my invention are set forth with particularly in 40 the appended claims. The invention itself however will best be understood from reference to the following specification when considered in connection with the accompanying drawing in which Fig. 1 represents diagrammatically a cross section of a spray device whereby my invention may be carried into effect, while Fig. 2 is a cross section of a modified form of spray torch.

Referring more particularly to the drawing, I have indicated at 1 an outer metal casing or 50 envelope spaced from an inner receptacle 2. Mounted within the latter is a heating chamber 3 spaced from the container 2 by a suitable insulating material 2' such as magnesium oxide. The heating chamber 3 consists of a cup-shaped graphite member 4 and a concentrically arranged

hollow graphite member 5 provided with a plurality of inclined openings 8. The member 5 surrounds an opening 6 in the bottom of the cup-shaped member 4 and extends a short distance above the upper end of the cup-shaped member. 60 The side and bottom walls of member 4 are provided with a plurality of ducts 7 which communicate with the opening 6 and with the member 5.

A graphite or tungsten pipe 9 is concentrically disposed within the member 5 and extends 65 through and beyond the latter member and envelope 1. The pipe 9 has a relatively large opening 10 adjacent the upper end of and within the member 5 providing an outlet through the pipe for the hot gas which flows through the heating chamber 3. A pair of insulating closure plugs 11 and 12 are fitted in the upper ends of members 4 and 5 respectively, while a graphite plug 13, fitted around the pipe 9, acts as a closure member for the opening 6, the plug being mounted 75 in that portion of opening 6 below the ducts 7.

The graphite member 5 and the central pipe 9 are provided with electrically conducting collars 14 and 15 respectively, adapted to be connected to a suitable source of electrical energy through 80 leads 16 and 17 which extend through insulating collars 18 mounted on the upper end of envelope 1.

In operation, a finely divided mixture of tungsten carbide and cobalt in suitable proportions 85 is fed into the upper end of pipe 9. A non-oxidizing gas such as carburetted hydrogen, pure nitrogen, pure argon, or nitrogen with a small percentage of hydrogen is supplied to the envelope 1 through a pipe 19. One portion of the 90 gas flows downwardly in the space between envelope 1 and container 2 and then outwardly through a series of openings 20 in the bottom of container 1 and adjacent the pipe 9. The remainder of the gas supplied to the envelope 95 flows downwardly through the ducts 7 into the opening 6 and around the inner graphite member 5 and finally through opening 10 into the pipe 9.

An electric current flows through the pipe 9 and graphite member 5 and heats these portions of the device to a temperature up to about 3000° C. At this temperature hydrogen reacts with graphite, forming hydrocarbons such as CH<sub>4</sub>, C<sub>2</sub>H<sub>2</sub> etc. so that even if hydrogen is employed the gas entering the tube 9 through the opening 10 is not pure hydrogen but contains a considerable percentage of hydrocarbons. The gases therefore which come in contact with the powdered mixture in tube 9 are not only non-oxidizing but non-decarbonizing as well. 110

The powdered mixture and gas flowing through the pipe 9 are heated to a high temperature and emerge as a jet or spray from the lower end of the pipe, the spray being surrounded by a shield 5 of non-oxidizing gas from the openings 20. The foundation metal or body 21 to be coated may be mounted on a movable table 22 adjacent the lower end of pipe 9. As the jet strikes body 21 it has a temperature above the melting point of 10 cobalt and iron, i. e. about 2200° C. and forms a thin layer of semi-plastic material which adheres to the supporting body 21.

While the electric current flowing through the members 4 and 5 and pipe 9 heats the powdered materials to the desired elevated temperature, an additional source of heat, such as a tungsten or graphite radiant heater, may be employed if desired to heat the body 21. An arrangement of this character is disclosed in Fig. 2 of the drawing, in which a hollow graphite heater 23 is provided at its upper end with a cap 24 and at its lower end with a screw-threaded graphite plug 25 which acts as a radiant heater.

A tungsten or graphite tube 26 extends centrally through the heater 23 and plug 25 and is insulated from cap 24 by a collar 27. Tube 26 is provided with an opening 28 within the member 23 to permit the flow of gas from heater 24 into the pipe 26. A coating 29 of insulating 30 refractory cement made by mixing zirconium oxide with sodium silicate and magnesium oxide is plastered on to the graphite heater 23. After drying, this insulating coating prevents excessive oxidation of the heater 23 and also limits the loss of heat into the surrounding atmosphere. A split graphite collar 30 surrounds the heater 23 and is connected to a wire 31. A similar wire 32 is connected to a conducting collar 33 mounted on tube 26. When wires 31 and 32 are connected 40 to a suitable source of electrical energy, current flows through the heater 23, plug 25 and tube 26 heating them to the desired temperature.

In operation, a powdered mixture such as described in connection with Fig. 1 is supplied to 45 the tube 26, while a gas such as hydrogen, nitrogen, argon or the like flows through pipe 34 connected to the heater 23 and to a suitable source of gas supply. The gas flows through the heater 23 and opening 28 into the tube 26 and diffuses 50 through the powdered material in the tube. The electric current flowing through the heater 23 and tube 26 heats the powdered materials and gas and plug 25 to an elevated temperature. Plug 25 acting as a radiant heater provides a 55 supplemental source of heat for the body 21 and the material deposited thereon.

The gas introduced into heater 23 provides a non-oxidizing and non-decarbonizing atmosphere for the deposition of the powdered materials on the body 21. The deposited material forms a semi-plastic layer on the supporting body 21, and when cooled is suitable for use as a wear 60 resistant surface or metal cutting tool.

What I claim as new and desire to secure by 65 Letters Patent of the United States, is:

1. The method of applying to a foundation metal a coating consisting mainly of a metal of

the 6th group of Mendelejeff's periodic table but containing appreciable but minor quantities of carbon and metal of the iron group, which comprises mixing the materials which comprise said coating in finely divided form, heating them to a relatively high temperature but below the melting point of the carbide of said metal of the 6th group, applying said mixture in the form of a spray and in a non-oxidizing and non-decarbonizing atmosphere to said foundation metal.

2. The method of applying to a foundation body a coating which consists mainly of tungsten but contains appreciable but minor quantities of carbon and metal of the iron group, which comprises mixing the materials which comprise said coating, heating them to a temperature below the melting point of tungsten carbide but sufficiently high to produce a semi-plastic material and applying said heated material to said foundation body in the form of a spray and in a non-oxidizing and non-decarbonizing atmosphere.

3. The method of applying a coating consisting of tungsten carbide and cobalt to a foundation metal which comprises mixing powdered tungsten carbide and cobalt introducing said mixture into a stream of non-oxidizing and non-decarbonizing gas, heating said gas and powdered mixture to a temperature of about 2200° C. and applying said mixture to a foundation metal.

4. The method of applying a coating consisting of tungsten carbide and cobalt to a foundation metal which comprises mixing powdered tungsten carbide and cobalt introducing said mixture into a stream of non-oxidizing gas, heating said gas and powdered mixture to a temperature of about 110 2200° C. and applying said mixture to a foundation metal.

5. A spray device comprising a casing, a hollow member extending through said casing, a pipe extending through and spaced from said member, means for heating said hollow member and pipe to an elevated temperature, means for circulating a gas through said hollow member and pipe and means whereby powdered materials may be supplied to said pipe.

6. The method of applying to a foundation body a coating consisting mainly of a hard metal carbide but containing an appreciable quantity of metal having a lower melting point than said carbide, which comprises mixing said carbide and metal in a finely divided condition, heating the mixture to a relatively high temperature but below the melting point of said carbide and applying said heated mixture to said foundation body in the form of a spray, said spray being surrounded by a shield of non-oxidizing gas.

7. A spray device comprising a hollow member of refractory material, an insulated pipe of refractory material extending through and spaced from said member, means whereby a non-oxidizing gas and powdered material may be supplied under pressure to said pipe, and means for passing an electric current through said pipe and member to thereby heat the material within said pipe to an elevated temperature.

PETER P. ALEXANDER.